

March 12, 1957

R. S. BABIARZ ET AL

2,785,081

PRODUCTION OF MULTI-COLORED DURABLE TIPPED  
EFFECTS ON EMBOSSED FABRICS

Filed Sept. 21, 1953

2 Sheets-Sheet 1

Fig. 1.



Fig. 2.



INVENTORS  
Raymond S. Babiarz  
Hilary Antoina Webley  
L. Synderfeld & Lechner  
ATTORNEYS

March 12, 1957

R. S. BABIARZ ET AL  
PRODUCTION OF MULTI-COLORED DURABLE TIPPED  
EFFECTS ON EMBOSSED FABRICS

2,785,081

Filed Sept. 21, 1953

2 Sheets-Sheet 2

Fig. 3.



Fig. 4.



Fig. 5.



Fig. 4a.



Fig. 5a

INVENTORS  
RAYMOND S. BABIARZ  
HILLARY ARTHUR WALLACE  
Symmetrode & Lechner  
ATTORNEYS

**1**

2,785,081

**PRODUCTION OF MULTI-COLORED DURABLE  
TIPPED EFFECTS ON EMBOSSED FABRICS**

Raymond S. Babiarz, Wilmington, and Hillary Arthur Wallace, New Castle, Del., assignors to Joseph Bancroft & Sons Company, Wilmington, Del., a corporation of Delaware

Application September 21, 1953, Serial No. 381,434

7 Claims. (Cl. 117—11)

This invention relates to the production of multi-colored durable tipped effects on embossed fabrics.

It has been known to produce durable embossed finishes and it has been suggested to durably tip embossed fabrics by applying color to the outermost portions or tips of the embossings. These, however, have been single color applications.

This invention is directed to producing durable multi-colored tipping effects in a simple and inexpensive manner.

In carrying out the invention, we first impregnate the fabric with a solution of thermosetting resin-forming materials, desirably in precondensate form, for which purpose any of the resins well known in this art for producing such durable embossed finishes may be employed, such, for example, as melamine type resins, urea type resins, and the like. The fabric is then squeezed to remove excess moisture and dried until it contains some moisture, preferably in the neighborhood of from 8% to 12%, or, alternatively, the fabric may be dried and conditioned by adding moisture, or dried and allowed to stand until it picks up moisture from the surrounding atmosphere by equilibrium, as is well known.

The fabric is now passed through the embossing calender, one bowl of which is composed of metal and has a pattern having a number of different distinct depths or levels engraved thereon, and the other of which is the so-called "soft bowl." The metal bowl is heated, usually from about 225° F. to about 350° F.

The thus specially embossed fabric is now ready for the tipping operation, which will be later described. At this point it will only be stated that the tipping machine (such, for example, as a Dornbusch #5 tipping machine) consists essentially of two rollers of suitable material which in this case, however, are mounted for adjustment toward and away from one another to vary the space therebetween. The color is applied to one of the rollers and is transferred to the tips of the face of the fabric, i. e., that face of the fabric which is next to the steel bowl in passage through the calender. As will later appear, the color paste also contains thermosetting resin forming material such as before mentioned.

After the fabric has been tipped, it is then subjected to a heat treatment to cure, set or polymerize the resins to the insoluble stage whereby to "fix" the embossed pattern and the color.

In the accompanying drawings (Figs. 1 and 2) we have diagrammatically illustrated, in exaggerated form, an embossed fabric typical of this invention, from which the mode of operation may be understood.

**2**

Fig. 3 is a flow sheet schematically illustrating one embodiment of the disclosed process for imparting multi-colored tipping effects to embossed patterns.

Figs. 4 and 5 are enlarged exaggerated schematic illustrations of two different passes by an embossed fabric, such as shown in Fig. 2, through a tipping machine. In Fig. 4 the tipping machine rollers are spaced apart so that only the highest level is color tipped and in Fig. 5 the tipping machine rollers are spaced apart so that the highest and intermediate levels are color tipped, as will be more fully described hereinafter.

Figs. 4a and 5a are schematic plan views of the fabric after passing through the tipping machines in Figs. 4 and 5 respectively.

It will be seen that in the case of the embossed fabric as illustrated in Figs. 1 and 2, the embossing has tips lying in four distinct levels, a topmost level A, a lower level B, a still lower level C, and a still lower level D which constitutes what might be called the base of the fabric. It will be understood, of course, that the pattern may otherwise be of any configuration desired. The number of passes through the tipping machine will depend upon the number of levels it is desired to color.

On the first run through the tipping machine (as for example shown in Fig. 4), the tipping rollers are spaced apart so as to exert light pressure only on tips lying in the outermost level A (Fig. 4a), the color being transferred from the printing roller as described. The fabric is now desirably dried. On the next run (schematically illustrated in Fig. 5) a different color may be applied to the printing roll; and the tipping rollers are now placed more closely together so that the color roll will reach the tips lying in the next lower level B and transfer the color. This is desirably followed by drying. In this run the tips in level A will, of course, be over-colored (Fig. 5a). On the next run, the rollers are set still more closely together so as to reach the tips of the next lower level C and again desirably dried. The tips of levels A and B will be over-colored by the color used in tipping the tips of level C. Usually level D which carries the base color of the fabric, is not colored by the tipping machine. The drying may be done, for example, by passage between hot steam plates or by a loop drier, so that enough drying is accomplished to prevent smearing during batching.

The procedure may be reversed, and the initial setting of the tipping rollers be made such as to reach the tips of level C and then adjusted to reach to the tips of level B, and again adjusted to reach to the tips of level A.

Very beautiful effects can thus be obtained, and these effects will be durable.

Curiously, we have found that although at the time of passage through the tipping machine, the resin with which the fabric has been impregnated before the embossing operation, is not yet cured, the embossed pattern and the physical deformation of the fibers of the yarns which have been imparted by the calender are not destroyed or impaired by the tipping operation. Hence, in the subsequent heat treatment or curing step, the curing of the resin in the fabric and in the paste, not only "fixes" the pattern and the physical deformation imparted by the embossing calender, i. e., so that they remain durable to repeated washings and dry cleanings, but also

## 3

renders the color tipping durable to washings and dry cleanings.

The paste containing the color pigment and the resin, is of the character largely used in conventional printing operations. Thus it may contain thickeners in addition to the resin, driers, softeners, water, and the like. Of course, the paste should be of a consistency such that it may be transferred to the tips without running or build up, as is well understood in this art.

It will also, of course, be understood that the impregnating solution and the paste may contain catalysts, usually an acid catalyst, also as well understood in this art.

*Example*

But one example will serve by way of illustration.

1. A pure bleached and scoured cotton fabric having the construction 39"-80/80-4.00 was impregnated with the following resin solution and frame dried to approximately 10% moisture content.

|                       |      |     |
|-----------------------|------|-----|
| Resloom HP            | lbs  | 40  |
| Resloom M-75          | do   | 40  |
| Aerotex H             | do   | 20  |
| PVA                   | do   | 5   |
| Catalyst AC           | do   | 10  |
| Total (water to make) | gals | 100 |

2. It was then embossed using a three level pattern at a speed of about 20 yds./min. and a temperature of 375° F. of the metal bowl of the embossing calender.

3. Tipped on the tipping machine using the following color formula:

|                              | Pounds |
|------------------------------|--------|
| PVA 72-60 (11% solution)     | 40     |
| Aerotex M-3 (melamine resin) | 12     |
| Aridye Padding Red B         | 7      |
| Ammonia                      | 1      |
| Ahcovel G                    | 2      |
| Catalyst AC                  | 1      |
| Water                        | 37     |
| Total                        | 100    |

The pressure setting of the pair of tipping rollers was first adjusted so as to cover the outermost level of the embossed fabric. This setting colored the top level of the embossing as well as the dotted effect of the lower level.

The speed was about 20 yds./min. and the fabric was dried after tipping in a continuous manner by passing between two hot steam plates.

4. The fabric was rerun through the same machine using the same printing formulation except the Aridye Padding Red B was replaced by Aridye Padding Blue 2G.

This time the pressure of the rollers was adjusted so as to color only the next level of the embossed fabric. Drying was similar to the previous run.

5. The fabric was cured for 3 minutes at 300° F., washed and dried in a slack (non-tension) drier.

The result was a durable two colored embossed fabric.

In the foregoing illustrative example "Resloom HP" is dimethylol melamine, "Resloom M-75" is a dimethylol trimethylol melamine (60% solids), "Aerotex H" is a cationic softener (a fatty chain modified melamine resin), "PVA" is polyvinyl alcohol, "Catalyst AC" is methyl hydroxy propanolamine hydrochloride, "Aerotex M-3" is dimethyl trimethylol melamine, "Aridye Padding Red B" is a red organic (phthalocyanine) pigment dispersion, "Aridye Padding Blue 2G" is a blue organic (Phthalocyanine) pigment dispersion and "Ahcovel G" is a s-di-[1-(2-stearoamidoethyl)] urea monoacetate.

While the fabric of the example is cotton, it will, of course, be understood that the process is applicable to other types, such, for example, as rayon, nylon, mixed goods, and the like.

For purposes of facilitating understanding of the in-

## 4

vention, the drawings have been greatly exaggerated and distorted. The levels are in reality only very shallow in depth, so that lateral shifting of the fabric, if any, with respect to the printing roll is negligible.

5. We claim:

1. The method of imparting durable multi-colored tipping effects to embossed fabrics which comprises first passing an embossed fabric through a color tipping machine to apply a heat hardenable resin paste of a first color to areas of the raised embossed portions of said fabric, which are temporarily compressed during the first tipping operation, passing the thus treated fabric through a color tipping machine to apply a heat hardenable resin paste of a second color to those areas of the raised embossed portions of the fabric which are thereby temporarily compressed during the second tipping operation, the degree of compression of the raised embossed pattern being different during the application of the first color than the degree of compression of the raised embossed pattern during the application of the second color, and thereafter heating the fabric to harden the resin.

2. The method of imparting durable multi-colored tipping effects to embossed fabrics which comprises imparting an embossed pattern effect to a fabric, temporarily compressing portions of the raised embossed pattern and simultaneously applying thereto in the compressed areas a heat hardenable resin paste of a first color, thereafter temporarily compressing portions of the raised embossed pattern and simultaneously applying thereto in the then compressed areas a heat hardenable resin paste of a second color, the degree of compression of the raised embossed pattern being different during the application of the first color than the degree of compression of the raised embossed pattern during the application of the second color, and thereafter heating the fabric to harden the resin.

3. The method of imparting durable multi-colored tipped embossed pattern effects to fabrics which comprises impregnating the fabric with a heat hardenable resin solution, drying the fabric to a moist condition, passing the moist fabric through an embossing calender thereafter, and before hardening of the resin to render the embossed effect durable, temporarily compressing portions of the raised embossed pattern and simultaneously applying thereto in the compressed areas a heat hardenable resin paste of a second color, the degree of compression of the raised embossed pattern being different during the application of the first color than the degree of compression of the raised embossed pattern during the application of the second color, and thereafter heating the fabric to harden the resin.

4. The method of imparting durable multi-colored tipping effects to embossed fabrics which comprises first passing an embossed fabric through a color tipping machine to apply a heat hardenable resin paste of a first color to areas of the raised embossed portions of said fabric, which are temporarily compressed during the first tipping operation, drying the fabric, passing the thus treated fabric through a color tipping machine to apply a heat hardenable resin paste of a second color to those areas of the raised embossed portions of the fabric which are thereby temporarily compressed during the second tipping operation, the degree of compression of the raised embossed pattern being different during the application of the first color than the degree of compression of the raised embossed pattern during the application of the second color, and thereafter heating the fabric to harden the resin.

5. The process of claim 2 wherein the fabric is embossed with a pattern in which the raised tip portions of the pattern lie in at least two distinct and differing levels, applying a first color to tips which lie at the highest level,

and thereafter applying a second color to the tips which lie at a lower level while over-coloring the previously colored high tips.

6. The process of claim 2 wherein the fabric is embossed with a pattern in which the raised tip portions of the pattern lie in at least two distinct and differing levels, applying the first color simultaneously to the tips which lie in at least two of the differing levels, and thereafter over-coloring with a different color only those tips which lie at a higher level.

7. An embossed fabric in which the raised portions of the embossed pattern have tips which lie in at least two

5

10

different and distinct levels with respect to the fabric ground and wherein the tips at different levels are colored with different durable colors.

**References Cited in the file of this patent**

**UNITED STATES PATENTS**

|           |              |               |
|-----------|--------------|---------------|
| 1,742,363 | Martinek     | Jan. 7, 1930  |
| 2,598,264 | Jones et al. | May 27, 1952  |
| 2,645,049 | Brown        | July 14, 1953 |
| 2,667,426 | Davis        | Jan. 26, 1954 |